

# UNITED STATES PATENT OFFICE.

MARTIN F. COOMES AND ARUNAH W. HYDE, OF LOUISVILLE, KENTUCKY.

## PROCESS OF CARBURIZING MALLEABLE CAST-IRON OR LOW-CARBON STEEL.

SPECIFICATION forming part of Letters Patent No. 422,119, dated February 25, 1890.

Application filed May 29, 1889. Serial No. 312,566. (Specimens.)

*To all whom it may concern:*

Be it known that we, MARTIN F. COOMES and ARUNAH W. HYDE, citizens of the United States, residing at Louisville, in the county 5 of Jefferson and State of Kentucky, have invented certain new and useful Improvements in the Process of Carburizing Malleable Cast-Iron or Low-Carbon Steel; and we do declare the following to be a full, clear, and exact de-  
10 scription of the invention, such as will enable others skilled in the art to which it appertains to make and use the same.

Our invention relates to the manufacture of steel; and its object is to effect a cheap and 15 rapid carburization of malleable cast-iron or of low-carbon steel by the use of certain carbon compounds which are readily decomposed by contact with the heated metal to be car-  
20 burized, whereby the carbon is set free and unites with the metal, thus converting the malleable cast-iron into steel or the low-car-  
bon steel into high-carbon steel.

To carry our invention into effect we em-  
25 ploy a bath composed of milk in any quan-  
tity, in which is placed the metal raised to a  
white heat, where it is allowed to remain while  
cooling. The heat from the metal decomposes  
the sugar and other carbonaceous compounds  
contained in the milk, and the carbon thus  
30 set free is absorbed by and chemically unites  
with the metal.

In our process any kind of milk, or its equiv-

alent condensed milk, may be used, and in  
any desired quantity to supply the requisite  
carbon, a deficiency or surplus of carbon af-  
fecting the extent and economy but not the  
completeness of the carburization. A quan-  
tity insufficient to carburize the whole mass  
will case-harden it, if case-hardening is de-  
sired; or the metal may be reheated and the  
process repeated.

In preparing the bath the milk may be  
mixed with water, and the following bath we  
find by experiment gives excellent results—  
namely, milk or condensed milk, one pound; 45  
water, one gallon.

If desired, the bath may be heated to any  
extent short of decomposing it before placing  
the heated metal in it.

Having fully described our invention, what 50  
we claim, and desire to secure by Letters Pat-  
ent, is—

In the manufacture of steel, the process of  
carburizing malleable cast-iron or low-carbon  
steel, which consists in immersing the metal 55  
raised to a white heat in milk, substantially  
as described.

In testimony whereof we affix our signatures  
in presence of two witnesses.

MARTIN F. COOMES.  
ARUNAH W. HYDE.

Witnesses:

W. E. BUCKEL,  
W. C. PETTY.